# EUROPEAN PATENT SPECIFICATION

(11) **EP 0 815 325 B1**
(45) Date of publication and mention of the grant of the patent: **31.07.2002**
(21) Application number: 96904198.7
(22) Date of filing: 01.03.1996
(51) Int. Cl.: E01B 11/46, E01B 31/12

(54) **IMPROVEMENTS IN AND RELATING TO STEEL RAILS AND METHODS OF PRODUCING THE SAME**
HERSTELLUNGSVERFAHREN FÜR EISENBAHNSCHIENEN AUS STAHL UND VERBESSERUNGEN DAZU
AMELIORATIONS APPORTEES AUX RAILS EN ACIER ET METHODES DE FABRICATION

(30) Priority: 20.03.1995 GB 9505567
(43) Date of publication of application: 07.01.1998
(73) Proprietor: Corus UK Limited, London SW1P 4WY (GB)
(72) Inventor: JERATH, Vijay, Aston Sheffield South Yorkshire S31 0GF (GB); CHAPMAN, John, Anthony, Doncaster South Yorkshire DN10 6JH (GB); PRICE, David, James, Rotherham South Yorkshire S65 1PB (GB)
(74) Representative: Fry, Alan Valentine
(86) International application number: GB9600458
(87) International publication number: WO9629469

(56) References cited:
- FR-A- 841 129
- FR-A- 2 642 087
- GB-A- 494 175
- ESVELD: "Modern Railway Track" 1989 , MRT PRODUCTIONS , DUISBURG (DE) XP002007196 166260 see page 170 - page 172 see page 102 - page 103

## Description

This invention relates to steel rails and to methods of producing the same. More especially, the invention relates to the production of high integrity long welded steel rails.

Railway tracks have traditionally comprised a plurality of rails connected together by bolts and fish plates. In use, such tracks have proved to be noisy, uneven and require considerable maintenance. More recently, individual rails have been welded together in continuous lengths thereby enabling higher train speeds to be achieved at relatively low noise and vibration levels. The welds between adjoining individual rails have, however, previously been subject to occasional bending fatigue failures from the foot of the rail caused *inter alia* by positive tensile loading stresses experienced by the rail foot during service.

One object of the present invention is to provide a high integrity long welded steel rail which exhibits a bending fatigue life commensurate with that of non-welded rail and an overall improved residual stress pattern across the weld HAZ profile. Another object is to provide a welded steel rail in which the bending fatigue strength of each weld is at least equal to if not greater than the fatigue strength of the parent rails joined by that weld. A further object is to produce a welded steel rail in which the presence of the welds is not apparent from a visual inspection (that is to say an invisibly welded rail). A further object is to provide a method or methods of manufacturing welded steel rail by which the objectives set out above can be achieved.

Typically a long welded rail is a length of the order of 100m to 300m or longer.

According to the present invention in one aspect there is provided a steel rail which comprises a plurality of individual rails welded together with any resulting excess material removed from the rail by a stripping process in which weld sites at and below the foot of each rail are subjected to grinding.

Document entitled Esveld: "Modern Railway Track" 1989 discusses various welding techniques for joining neighbouring rails of a continuous track. Stripping of weld material from the rail foot and foot undersurface is, however, not contemplated.

Each weld site may be coated with a corrosion inhibiting material. Such coating may be applied to the rail foot and or the rail web and/or the rail head. The coating may, of course, alternatively be applied to the entire weld site.

Welding may be by flash butt welding. Other welding processes may however be employed.

In another aspect, the present invention provides a method of producing a welded steel rail which comprises the steps of welding individual rails together, removing any resulting excess material from the weld sites and subsequently subjecting the weld sites at and below the foot of each rail to air cooling, grinding and peening.

As-rolled rail grades such as 700 and 900 (BS11 Normal quality and Grade A/AREA) achieve weld HAZ hardness levels similar to those of the parent rails following natural air cooling of the welds in still air. These rails following welding are, therefore, not normally subjected to accelerated cooling. It has, however, been found advantageous to increase the hardness/strength, in particular, of the welded rail foot by accelerated cooling with a view to improving the bending fatigue strength of the welded rail.

Accelerated cooling may be achieved by applying air, air mist or water under pressure independently to the head and/or the web and/or the foot of the rail at each weld site. Typically, forced cooling is applied through the appropriate phase transformation temperature range, eg austenite to pearlite, austenite to bainite or austenite to martensite. Typically cooling is initiated at a temperature within the high temperature austenite phase of the steel and stopped at a temperature deemed suitable for the completion of a given phase transformation. Accelerated cooling may typically be effected for a period of between 30 and 120 seconds. Forced cooling may be effected by either individual hoods or nozzles positioned above and to the sides of the head of the rail, opposite each web of the rail, and below the foot surface of the rail, each independent hood or nozzle being supplied with air, air mist or water under pressure from a common or a different source. Thus cooling may be effected to, for example, only the rail head,foot or web, or to the entire rail.

Fine grinding or surface material removal by another technique of the welded regions may be applied to the head and/or the underside of the rail foot and/or to the web of the rail. Invisibly welding of a rail entails, however, grinding or other surface material removal all around the rail profile after welding of the individual rails together.

Robotic material removal techniques may be employed. Surface material removal may be effected either cold or at a temperature below the austenite temperature of the steel from which the rail is produced. Sensors may be provided to ensure that the required material removal depth and surface finish are achieved.

Peening may, for example, be by a shot or a hammer peening process and may be applied to the underside of the foot of the rail and/or to the head and/or web of the rail or to the entire welded or unwelded (ie parent rail) rail profile.

Peening may be achieved by directing a peening medium under pressure independently to the foot and/or head and/or web of the rail at each weld site. The depth of the residual compressive stress layer may be, for example, between 0.75mm and 1mm and the compressive stresses achieved may be, for example, of the order of 60% to 80% of the yield strength of the rail material in compression. Peening is generally carried out at a temperature below the stress relieving temperature of the steel from which the rail is produced, typically below 250°C.

The invention will now be described by way of example with reference to the accompanying diagrammatic drawings in which:-
Figure 1 is a transverse section taken through a steel rail and shows substantially typical fatigue initiation sites in the foot of the rail associated with bending fatigue failures.;
Figures 2 and 3 are side views of accelerated cooling apparatus in accordance with the present invention;
Figure 4 graphically illustrates the effect of forced cooling on flash butt weld HAZ hardness of fully pearlitic plain carbon rails;
Figure 5 graphically illustrates the generation of residual stress in a shot peened steel after surface grinding and showing beneficial compressive stress produced following fine grinding;
Figure 6 is a side view of peening apparatus in accordance with the invention;
Figure 7 graphically illustrates induced compressive surface stresses and tensile stresses in a shot peened steel material;
Figure 8 graphically illustrates longitudinal residual stress distributions in a roller straightened steel rail, a flash butt welded rail and a ground and shot peened welded rail; and
Figure 9 graphically compares bending fatigue strengths of a parent rail, a normal production weld, a weld ground all around, a weld ground all around and shot peened and a normal production weld after shot peening.

The welded rail illustrated in Figure 1 has a head 1, a web 2 and a foot 3. Typical bending fatigue initiation sites in the illustrated welded rail are indicated by reference numbers 4, 5 and 6. As will be seen, all of these fatigue initiation sites are located in the foot region of the rail. Of the sites illustrated, site 4 located in the base of the foot 3 is found to be the most prevalent, and is generally caused by maximum tensile stresses occasioned by the bending forces generated during service.

As mentioned previously, it is an object of this invention to provide a high integrity long welded steel rail having bending fatigue life and wear performance at least as good, if not better than, those of rails manufactured currently. This objective is currently achieved by flash butt welding (otherwise called electrical resistance welding) individual steel rails together, stripping the resulting flash from the weld sites and then subjecting the weld sites to one, more than one or indeed all of the process steps of natural air or forced cooling, fine grinding and peening. These process steps will now be discussed in more detail.

Flash butt welding is a process in which the rail ends to be joined together are held between water cooled copper grips, which act as both clamps and electrodes. The first stage in the flash butt welding sequence is generally termed the "Burn-Off" or the "Pre-flashing" stage. During this stage, the rail ends are separated slightly and arcing/flashing is initiated between them in order to square up the rail ends. "Burn-Off" times are typically between 5 and 10 seconds, with 1-5mm of platten movement. The next stage in the welding sequence is the preheating stage. The main aim of the preheating stage is to heat the rail ends to a sufficient temperature so that flashing initiates easily, and a suitable temperature gradient is achieved in the rail ends, prior to the onset of the final flashing sequence. Preheating is generally achieved by bringing the rail ends into contact, and allowing a high current to flow across the rail ends. The rail ends are brought together and allowed to heat by means of resistance heating.

In between each preheating cycle a short period of flashing is generally allowed to occur in order to maintain rail end squareness. This is followed by the final "flashing" stage. During this stage the rail interfaces become molten, and the correct conditions for the final upset or the forging stroke are achieved. The moving head of the welding machine during this stage is accelerated parabolically, with the resultant increase in the frequency and number of flashing ruptures or arcs across the weld interface. This ensures that the oxygen content at the weld interface is reduced sufficiently to give a semi-protective atmosphere. The primary purpose of the final flashing stage is to generate enough heat to produce a plastic zone that permits adequate upsetting. A total flashing distance of between 9 and 15 mm, over a period of 5 to 10 seconds, is typically employed for rails. Immediately following the final flashing stage, the movable platten of the welding machine is accelerated so that the rail ends are butted together either under a constant platten speed or under impact loading of up to 600 kN. The load is calculated to give a pressure at the weld interface of approximately 50-60 N/mm², to ensure adequate weld consolidation. The welding current is generally supplied during the initial part of the forging operation to avoid oxidation at the weld interface. During welding of rails, a typical forging distance of between 12 and 20 mm is generally employed. Following the completion of the forging stroke, the molten and soft steel is forced out of the weld joint. This extruded material, generally termed "flash" is then removed quickly by means of an automatic weld upset removal tool.

One recognised advantage of flash butt welding is that good quality welds requiring no external weld metal can be produced in a relatively short period of time, typically within 45 to 90 seconds.

Other welding techniques may be employed, e.g. squeeze welding.

Accelerated forced cooling is a process for rapidly and controllably reducing the temperature of a product. When used in the context of the present invention, the weld sites, for example, of heat treated, plain carbon pearlitic rail are cooled through the austenite to pearlite transformation temperature range (typically from 700°C to 500°C) at, for example, up to 7°C/second. Enhanced cooling of the weld sites at the correct rate produces weld HAZ hardness levels which match those of the parent plain carbon heat treated rail. The effect of different forced cooling rates on HAZ hardness can be seen from Figure 4. Thus, the effect of independent forced air cooling of the welded rail head, web and foot weld sites is effected with a view to increasing the hardness and wear resistance of the rail head, to improve the rolling contact fatigue life of the welded rail head and bending fatigue strength of the rail foot, and to improve the overall residual stress pattern across the weld HAZ profile.

As-rolled rail grades such as 700 and 900 (BS11 Normal quality and Grade A/AREA) achieve weld HAZ hardness levels similar to those of the parent rails following natural air cooling of the welds in still air. These rails following welding are, therefore, not normally subjected to accelerated cooling. It has, however, been found advantageous to increase the hardness/strength, in particular, of the welded rail foot by accelerated cooling with a view to improving the bending fatigue strength of the welded rail.

Apparatus for effecting forced cooling is illustrated in Figures 2 and 3. In Figure 2 the cooling medium is air and in Figure 3 water. As shown in Figure 2, cooling hoods 7 supported within a frame 9 and each connected by conduits 8 to a source of air under pressure are positioned above and to each side of the rail head, alongside each rail web and below the rail foot. The arrangement is such that one or more (or indeed all) of the hoods may be connected to direct cooling air under pressure onto the adjoining rail surface. The flow of air through the conduits is individually controlled by means of valves positioned, for example, within the conduits.

In the arrangement illustrated in Figure 3, water is supplied under pressure via nozzle 11 to a manifold 12. Cooling water is selectively projected onto the head, web and/or foot of the rail by nozzles 14.

The effect of forced cooling on HAZ hardness of fully pearlitic plain carbon rails is illustrated graphically in Figure 4.

Surface grinding of the welded rail head is carried out as a routine production procedure to match the profile of the parent rail. Alternatively, surface material removal from the rail head may be carried out by another technique. Additional surface grinding (or surface material removed by another technique) to the web and foot of the rail may be effected in the present invention with a view to rendering the weld invisible to the eye. Beneficial grinding (or other method of surface material removal) of the weld sites may be effected to reduce the number of potential fatigue initiation sites, eg surface pitting and by removing all traces of weld flash and decarburized layer from each weld site, particularly that from the rail foot which experiences tensile loading stresses during service.

Surface material removal, for example, by grinding may be carried out by use of a robotic grinder which automatically fine grinds selected parts or each entire weld site of the rail.

Grinding may be effected either cold or at a temperature below the austenite temperature of the rail, typically 700°C. Sensors may be provided to ensure that the required grinding depth and surface finish are achieved.

A graph illustrating the generation of residual stress in a 4340 steel after surface grinding is shown in Figure 5. The beneficial compressive stress introduced by fine grinding is to be noted.

In addition fine grinding or other surface material removal technique particularly of the base of the welded rail foot also enables a full in-line automatic non-destructive testing (NDT) and/or additional alternative manual inspection of the welded rail to be carried out. Thus, the rail head, web and foot can readily be ultrasonically tested to a required specification, the rail foot base can be eddy current tested, and the flatness of the rail running surface and the rail head sides can be inspected. Also, manual ultrasonic inspection of each weld site for transverse defects can be effected with considerable ease.

Peening may be effected by, for example, a shot or hammer peening process.

Shot peening is a cold working process in which the surface of a part is bombarded with small spherical media called shot. Each piece of shot striking the material acts as a tiny peening hammer, imparting to the surface a small indentation or dimple. In order for the dimple to be created, the surface fibres of the material must be yielded in tension. Below the surface, the fibres try to restore the surface to its original shape, thereby producing below the dimple, a hemisphere of cold-worked material highly stressed in compression. Overlapping dimples develop an even layer of metal in residual compressive stress. It is known that a compressively stressed zone increases the initiation time required for a crack to form for a given applied tensile stress range. Since nearly all fatigue and stress corrosion failures originate at the surface of a part, compressive stresses induced by shot peening provide considerable increases in part life. The maximum compressive residual stress produced at or under the surface of a part by shot peening is at least as great as half the yield strength of the material being peened. Many materials will also increase in surface hardness due to the cold working effect of shot peening.

Shot peening apparatus for use, for example, with the invention is schematically illustrated in Figure 6. This apparatus comprises a plurality of nozzles 15 positioned above, below and to the sides of the rail. Each nozzle is mounted on a frame 16 and is connected to receive a source of gas under pressure and shot. Each nozzle can be independently controlled whereby the head, web and foot of the rail can be together or selectively peened.

Benefits obtained by shot peening are the result of the effect of the compressive stress and the cold working induced. In the present invention, peening is effected to welded rail and/or unwelded rail, i.e. parent rail, thereby creating compressive stresses which act to minimise the onset of crack initiation during service.

In one example, shot peening to the specification MIL-S-13165C was applied to the rails in the present invention. This peening process employed a shot size of 1.375mm (MI 550) at an intensity of 0.012-0.014C. A range of shot sizes and intensity levels can, nevertheless, be employed to obtain beneficial compressive stresses.

Typical compressive stresses achieved by the process are, for example, of the order of 60 to 80% of the yield strength of the rail material in compression. The depth of the residual compressive layer produced by peening is, for example, typically between 0.75mm and 1.0mm. Peening is generally effected at a temperature below the stress relieving temperature of the steel from which the rail is produced, typically below 250°C.

The effect of induced compressive and tensile stresses in a shot peened material with no external load is illustrated in Figure 7 of the drawings and Figure 8 graphically illustrates longitudinal residual stress distribution in a conventional rail, a weld and a shot peened weld.

A comparison of the results of 4-point bend fatigue testing of conventional rails and welded rails in accordance with the present invention can be seen from Figure 9. This Figure shows that the high integrity welds produced in accordance with this invention and labelled "3" "4" and "5" possess bending fatigue strength levels significantly in excess of that of the parent or unwelded rail labelled "1".

Bending fatigue data for as-rolled welded rails which have been either ground or ground and shot peened have been found to be at least as good as, if not better than, those of the parent rails. These rails have shown similar overall trends to those observed in the case of mill heat treated rails (MHT) as exemplified in Figure 9.

The techniques mentioned above concerning the production of high integrity invisible welds may also be applied readily to all grades of as-rolled and heat treated pearlitic rails and to any other additional rail grades developed in the future.

In addition, the techniques mentioned above may be applied readily to the bainitic and martensitic steels disclosed in our co-pending patent applications 950097.1 and 9313060.

It will be appreciated that the foregoing is merely exemplary of rails in accordance with the invention and that modifications can readily be made thereto without departing from the scope of the invention as defined in the claims.

## Claims

1. A steel rail which comprises a plurality of individual rails welded together with any resulting excess material removed from the rail by a stripping process in which weld sites at and below the foot of each rail are subjected to grinding.

2. A rail as claimed in claim 1 wherein the weld sites at and below the foot of each rail are subjected to natural air cooling.

3. A rail as claimed in claim 1 wherein the weld sites at and below the foot of each rail are subjected to independent accelerated cooling.

4. A rail as claimed in any one of the preceding claims wherein the weld sites at and below the foot of each rail are subjected to peening.

5. A rail as claimed in any one of the preceding claims wherein each weld site is coated with a corrosion inhibiting material.

6. A method of producing a welded steel rail which comprises the steps of welding individual rails together, removing any resulting excess material from the weld sites and subsequently subjecting the weld sites at and below the foot of each rail to air cooling, grinding and peening.

7. A method as claimed in claim 6 wherein the weld sites are subjected to accelerated cooling by applying air, air mist or water under pressure to and below the foot of each rail.

8. A method as claimed in claim 7 wherein accelerated cooling is effected for a period of between 30 and 120 seconds.

9. A method as claimed in claim 7 or claim 8 wherein forced cooling is effected around each entire weld site of each rail by directing cooling medium through nozzles positioned above and to the sides of the head of the rail, opposite each web of the rail, and below the foot surface of each rail.

10. A method as claimed in claim 6 wherein peening is effected around the entire weld site of each rail by directing a peening medium under pressure to and below the foot, the head and web of each rail.

11. A method as claimed in claim 10 wherein the depth of the residual compressive stress layer achieved is between 0.75mm and 1mm and the compressive stresses achieved are between 60% to 80% of the yield strength of the rail material in compression.

12. A rail as claimed in claim 10 or Claim 11 wherein peening is carried out at a temperature below the stress relieving temperature of the steel from which the rail is produced.

## Patentansprüche

1. Stahlschienenstrang, bestehend aus mehreren einzelnen miteinander verschweißten Schienen, bei dem irgendein sich ergebendes überschüssiges Material von dem Schienenstrang durch ein Abstreifverfahren entfernt wird, bei dem Schweißstellen am Fuß einer jeden Schiene und darunter einem Schleifvorgang unterworfen werden.

2. Schienenstrang nach Anspruch 1, bei welchem die Schweißstellen an dem Schienenfuß jeder Schiene und darunter einer Umgebungsluftkühlung ausgesetzt werden.

3. Schienenstrang nach Anspruch 1, bei welchem die Schweißstellen an und unter dem Schienenfuß jeder Schiene einer unabhängigen Beschleunigungskühlung unterworfen werden.

4. Schienenstrang nach einem der vorhergehenden Ansprüche, bei welchem die Schweißstellen an und unter dem Schienenfuß jeder Schiene einem Hämmervorgang unterworfen werden.

5. Schienenstrang nach einem der vorhergehenden Ansprüche, bei welchem jede Schweißstelle mit einem Korrosionsschutzmaterial überzogen ist.

6. Verfahren zur Erzeugung eines verschweißten Schienenstrangs mit den folgenden Schritten: es werden einzelne Schienen miteinander verschweißt; es wird das sich ergebende überschüssige Material von der Schweißstelle entfernt, und es werden danach die-Schweißstellen an und unter dem Schienenfuß jeder Schiene einer Luftkühlung, einem Schleifvorgang und einem Hämmervorgang unterworfen.

7. Verfahren nach Anspruch 6, bei welchem die Schweißstellen einer Beschleunigungskühlung unterworfen werden, indem Luft, Luftnebel oder Wasser unter Druck auf den Fuß jeder Schiene und unter diesen gespritzt wird.

8. Verfahren nach Anspruch 7, bei welchem die Beschleunigungskühlung während einer Dauer zwischen 30 und 120 Sekunden durchgeführt wird.

9. Verfahren nach Anspruch 7 oder Anspruch 8, bei welchem eine Zwangskühlung um die gesamte Schweißstelle einer jeden Schiene bewirkt wird, indem ein Kühlmedium über Düsen gerichtet wird, die über dem Kopf der Schiene und seitlich zu diesem sowie auf gegenüberliegenden Seiten des Schienensteges und unter der Oberfläche des Schienenfußes jeder Schiene angeordnet sind.

10. Verfahren nach Anspruch 6, bei welchem der Hämmervorgang über die gesamte Schweißstelle jeder Schiene dadurch bewirkt wird, daß ein Kugelstrahl unter Druck auf den Schienenfuß und unter diesen sowie auf den Kopf und den Steg einer jeden Schiene gerichtet wird.

11. Verfahren nach Anspruch 10, bei welchem die Tiefe der erreichten Restdruck-Beanspruchungsschicht zwischen 0,75 mm und 1 mm dick ist und die sich ergebenden Druckbeanspruchungen zwischen 60% und 80% der Streckfestigkeit des unter Druck stehenden Schienenmaterials liegen.

12. Schienenstrang nach den Ansprüchen 10 oder 11, bei welchem der Hämmervorgang bei einer Temperatur durchgeführt wird, die unter der Spannungsentlastungs-Temperatur des Stahls liegt, aus dem die Schiene erzeugt ist.

## Revendications

1. Rail en acier qui comprend plusieurs rails individuels soudés les uns aux autres, toute matière en excès résultant de la soudure étant éliminée du rail via un procédé d'épuration dans lequel les sites de soudage à la base de chaque rail et en dessous de ladite base sont soumis à un meulage.

2. Rail selon la revendication 1, dans lequel les sites de soudage à la base de chaque rail et en dessous de ladite base sont soumis à un refroidissement naturel à l'air.

3. Rail selon la revendication 1, dans lequel les sites de soudage à la base de chaque rail et en dessous de ladite base sont soumis à un refroidissement accéléré indépendant.

4. Rail selon l'une quelconque des revendications précédentes, dans lequel les sites de soudage à la base de chaque rail et en dessous de ladite base sont soumis à un écrouissage.

5. Rail selon l'une quelconque des revendications précédentes, dans lequel chaque site de soudage est enduit d'une matière inhibant la corrosion.

6. Procédé de fabrication d'un rail en acier soudé qui comprend les étapes consistant à souder les uns aux autres des rails individuels, à éliminer la matière en excès résultante des sites de soudage et à soumettre ensuite les sites de soudage à la base de chaque rail et en dessous de ladite base à un refroidissement à l'air, à un meulage et à un écrouissage.

7. Procédé selon la revendication 6, dans lequel les sites de soudage sont soumis à refroidissement accéléré en appliquant de l'air, un brouillard d'air ou de l'eau sous pression sur la base de chaque rail et en dessous de ladite base.

8. Procédé selon la revendication 7, dans lequel on procède à un refroidissement accéléré pendant un laps de temps entre 30 et 120 secondes.

9. Procédé selon la revendication 7 ou 8, dans lequel on procède à un refroidissement forcé autour de chaque site complet de soudage de chaque rail en dirigeant un milieu de refroidissement à travers des buses qui ont été positionnées au-dessus et sur les côtés de la tête du rail, face à chaque âme du rail et en dessous de la surface de la base de chaque rail.

10. Procédé selon la revendication 6, dans lequel on effectue l'écrouissage autour du site de soudage complet de chaque rail en dirigeant un milieu d'écrouissage sous pression en direction de la base de chaque rail et en dessous de cette dernière, en direction de la tête et en direction de l'âme de chaque rail.

11. Procédé selon la revendication 10, dans lequel la profondeur de la couche de contraintes rémanentes de compression que l'on obtient se situe entre 0,75 mm et 1 mm et les contraintes de compression que l'on obtient représentent entre 60 % et 80 % de la résistance à la déformation de la matière du rail par compression.

12. Rail selon la revendication 10 ou 11, dans lequel on effectue l'écrouissage à une température inférieure à la température de relaxation des contraintes de l'acier à partir duquel le rail a été fabriqué.
